

UNITED STATES PATENT OFFICE

**2,656,351**

# TRINUCLEAR DYES CONTAINING A 5-THIAZOLIDONE NUCLEUS

Per Aubert, Oslo, Norway, and Roy A. Jeffreys and Edward B. Knott, Harrow, England, assignors to Eastman Kodak Company, Rochester, N. Y., a corporation of New Jersey

**No Drawing. Application March 2, 1951,  
Serial No. 220,332**

**8 Claims. (Cl. 260—240.1)**

1

This invention relates to trinuclear dyes containing a 5-thiazolidone nucleus and to methods for preparing them. More particularly, this invention relates to trinuclear dyes useful in altering the sensitivity of photographic silver halide emulsions.

Trinuclear dyes obtained from merocyanine dyes containing a rhodanine nucleus have previously been described. Fry et al. U. S. Patent 2,388,963, dated November 13, 1945. Such dyes, in certain cases, can advantageously be employed in altering the sensitivity of photographic silver halide emulsions.

We have now found a new class of trinuclear dyes which can also be used in altering the sensitivity of photographic silver halide emulsions.

It is, therefore, an object of our invention to provide new trinuclear dyes. A further object is to provide methods for preparing these dyes. Still another object is to provide photographic silver halide emulsions containing these new dyes, and methods for preparing these emulsions. Other objects will become apparent from a consideration of the following description and examples.

According to our invention we provide tri-nuclear dyes selected from those represented by the following two general formulas:



and



wherein R, R<sub>1</sub>, and R<sub>2</sub> each represents an alkyl group, such as methyl, ethyl, isopropyl, n-propyl, n-butyl, isobutyl, n-amyl, n-heptyl, n-octyl,  $\beta$ -hydroxyethyl,  $\beta$ -acetoxyethyl, etc. groups (e. g. an alkyl group of the formula C<sub>m</sub>H<sub>2m+1</sub> wherein  $m$  represents a positive integer from 1 to 8), and R<sub>1</sub> can, in addition, represent alkyl groups, such as the cycloalkyl groups, e. g. cyclopropyl, cyclobutyl, cyclopentyl, cyclohexyl, etc. groups (e. g. cycloalkyl groups containing from 3 to 6

2

carbon atoms in the cycloalkyl ring), *e* and *n* each represents a positive integer from 1 to 2, *d* represents a positive integer from 1 to 3, *X* represents an anion, such as  $\text{Cl}^-$ ,  $\text{Br}^-$ ,  $\text{I}^-$ ,  $\text{ClO}_4^-$ ,  $\text{p-CH}_3\text{C}_6\text{H}_4\text{SO}_3^-$ ,  $\text{C}_6\text{H}_5\text{SO}_3^-$ ,  $\text{CH}_3\text{COO}^-$ ,  $\text{-SCN}^-$ , etc., *L* represents a methine group, *Z* and *Z*<sub>1</sub> each represents the non-metallic atoms necessary to complete a heterocyclic nucleus containing from five to six atoms in the heterocyclic ring, such as those selected from the group consisting of those of the thiazole series (e. g. thiazole, 4 - methylthiazole, 4 - phenylthiazole, 5-methylthiazole, 5-phenylthiazole, 4,5 - dimethylthiazole, 4,5-diphenylthiazole, 4 - (2 - thiienyl)-thiazole, etc.), those of the benzothiazole series (e. g. benzothiazole, 4-chlorobenzothiazole, 5-chlorobenzothiazole, 6-chlorobenzothiazole, 7-chlorobenzothiazole, 4-methylbenzothiazole, 5-methylbenzothiazole, 6-methylbenzothiazole, 5-bromobenzothiazole, 6 - bromobenzothiazole, 4-phenylbenzothiazole, 5 - phenylbenzothiazole, 4-methoxybenzothiazole, 5 - methoxybenzothiazole, 6-methoxybenzothiazole, 5-iodobenzothiazole, 6-iodobenzothiazole, 4 - ethoxybenzothiazole, 5 - ethoxybenzothiazole, tetrahydrobenzothiazole, 5,6-dimethoxybenzothiazole, 5,6 - dioxymethylenebenzothiazole, 5 - hydroxybenzothiazole, 6 - hydroxybenzothiazole, etc.), those of the naphthothiazole series (e. g.  $\alpha$ -naphthothiazole,  $\beta$ -naphthothiazole, 5-methoxy -  $\beta$  - naphthothiazole, 5-ethoxy- $\beta$ -naphthothiazole, 8 - methoxy- $\alpha$ -naphthothiazole, 7-methoxy- $\alpha$ -naphthothiazole, etc.), those of the thionaphtheno-7',6',4,5-thiazole series (e. g. 4'-methoxythionaphtheno-7',6',4,5-thiazole, etc.), those of the oxazole series (e. g.

4-methyloxazole, 5-methyloxazole, 4-phenyloxazole, 4,5-diphenyloxazole, 4-ethyloxazole, 4,5-dimethyloxazole, 5-phenyloxazole, etc.), those of the benzoxazole series (e. g. benzoxazole, 5-chlorobenzoxazole, 5-methylbenzoxazole, 5-phenylbenzoxazole, 6-methylbenzoxazole, 5,6-dimethylbenzoxazole, 4,6 - dimethylbenzoxazole, 5 - methoxybenzoxazole, 5-ethoxybenzoxazole, 5-chlorobenzoxazole, 6-methoxybenzoxazole, 5-hydroxybenzoxazole, 6-hydroxybenzoxazole, etc.), those

of the naphthoxazole series (e. g.  $\alpha$ -naphthoxazole,  $\beta$ -naphthoxazole, etc.), those of the selenazole series (e. g. 4-methylselenazole, 4-phenylselenazole, etc.), those of the benzoselenazole series (e. g. benzoselenazole, 5 - chlorobenzoselenazole, 5 - methoxybenzoselenazole, 5 - hydroxybenzoselenazole, tetrahydrobenzoselenazole, etc.), those of the naphthoselenazole series (e. g.  $\alpha$ -naphthoselenazole,  $\beta$ -naphthoselenazole, etc.), those of the naphthoselenazole series (e. g.  $\alpha$ -methylthiazoline, etc.), those of the 2-quinoline series (e. g. quinoline, 3-methylquinoline, 5-methylquinoline, 7-methylquinoline, 8-methylquinoline, 6-chloroquinoline, 8-chloroquinoline, 6-methoxyquinoline, 6-ethoxyquinoline, 6-hydroxyquinoline, 8-hydroxyquinoline, etc.), those of the 4-quinoline series (e. g. quinoline, 6-methoxyquinoline, 7-methylquinoline, 8-methylquinoline, etc.), those of the 1-isoquinoline series (e. g. isoquinoline, 3,4-dihydroisoquinoline, etc.), those of the 3-isoquinoline series (e. g. isoquinoline, etc.), those of the 3,3-dialkylindolenine series (e. g. 3,3-dimethylindolenine, 3,3,7-trimethylindolenine, etc.), the pyridine series (e. g. pyridine, 5-methylpyridine, etc.), etc., and Q represents the non-metallic atoms necessary to complete a heterocyclic nucleus containing from five to six atoms in the heterocyclic ring, such as those selected from the group consisting of a thiazolone nucleus, for example, a 2,4(3,5)-thiaoledione nucleus, such as 2,4(3,5)-thiaoledione, 3-ethyl-2,4(3,5)-thiaoledione, 3-phenyl-2,4(3,5)-thiaoledione or 3-naphthyl-2,4(3,5)-thiaoledione nuclei, a 2-thio-2,4(3,5)-thiaoledione (a rhodanine) nucleus, such as 3-alkyl-2-thio-2,4(3,5)-thiaoledione (3-alkylrhodanine), 3 - phenyl-2-thio-2,4(3,5) - thiaoledione (3 - phenylrhodanine), 3 - naphthyl-2-thio-2,4(3,5) - thiaoledione (3-naphthylrhodanine) nuclei or 3-(1-benzothiazyl)-2-thio - 2,4(3,5)-thiaoledione (3-(1-benzothiazyl)-rhodanine) nuclei, a 2-thio-2,5(3,4)-thiaoledione nucleus, such as 3-methyl-2-thio-2,5(3,4) - thiaoledione, 3-ethyl-2-thio-2,5(3,4)-thiaoledione, 3-n-heptyl-2,5(3,4)-thiaoledione, 3-cyclohexyl-2,5(3,4)-thiaoledione, etc., a 2-alkylmercapto-4(5)-thiazolone nucleus, such as 2-ethylmercapto-4(5)-thiazolone, a thiazolidone nucleus, such as 4-thiazolidone or its 3-alkyl-3-phenyl or 3-naphthyl derivatives, a 2-alkyl-phenylamino-4(5)-thiazolone nucleus, or a 2-phenylamino-4(5)-thiazolone nucleus; an oxazolone nucleus, for example, a 2-thio-2,4(3,5)-oxazolone nucleus, such as a 3-alkyl-2-thio-2,4(3,5)-oxazolone nucleus; an imidazolone nucleus, for example a 2,4(3,5)-imidazolone nucleus, such as 2,4(3,5)-imidazolone (hydantoin) or its 3-alkyl, 3-phenyl or 3-naphthyl derivatives as well as its 1,3-dialkyl, 1-alkyl-3-phenyl, 1-alkyl-3-naphthyl, 1,3 - diphenyl, etc., derivatives, a 2-thio-2,4(3,5)-imidazolone nucleus, such as 2-thio-2,4(3,5)-imidazolone (2-thiohydantoin) or its 3-alkyl, 3-phenyl or 3-naphthyl derivatives as well as its 1,3-dialkyl, 1-alkyl-3-phenyl, 1-alkyl-3-naphthyl, 1,3-diphenyl, etc., derivatives, a 2-alkylmercapto-5(4)-imidazolone, such as 2-propylmercapto-5(4)-imidazolone; a thionaphthenone nucleus, such as 2-(1) - thionaphthenone or 1(2)-thionaphthenone, a pyrazolone nucleus, an oxindole nucleus, such as 2,3-dihydro-3-ketoindole, and like five-membered heterocyclic nuclei, a 2,4,6-triketohexahydropyrimidine nucleus, for example barbituric acid or 2-thiobarbituric acid, as well as their 1-alkyl or 1,3-dialkyl derivatives; a 3,4-dihydro-2(1)-quin-

alone nucleus, such as 3,4-dihydro-2(1)-quino lone (dihydrocarbostyryl); a 3,4 dihydro-2(1)-quinoxalone nucleus, such as 3,4-dihydro-2(1)-quinoxalone (oxydihydroquinoxaline); 3-phenomorpholone (1,4,2-benzoxazine-3(4)-one or benzo- $\beta$ -morpholone) nuclei; 1,4,2-benzothiazine-3(4)-one (ketodihydrobenzoparathiazine) nuclei, and the like six-membered heterocyclic nuclei. The dyes wherein Q represents the non-metallic atoms necessary to complete a heterocyclic nucleus containing five atoms in the heterocyclic ring, three of said atoms being carbon atoms, one of said atoms being a nitrogen atom, and the other of said atoms being a sulfur atom, a nitrogen atom, or an oxygen atom, have been found to be especially well adapted to the manufacture of photographic emulsions, we have found.

The new trinuclear dyes represented by Formula I above can advantageously be prepared by condensing a compound selected from those represented by the following general formula:



wherein R, R<sub>1</sub>, L, n, d, and Z have the values set forth above, and R<sub>2</sub> represents an alkyl group, such as methyl, ethyl, n-hexyl, etc. groups, and X<sub>1</sub> represents an anion, such as those represented by X above, for example, with a compound selected from those represented by the following general formula:



wherein Q has the values set forth above.

The new trinuclear dyes represented by Formula II above can advantageously be prepared by condensing a compound selected from those represented by Formula III above with a cyclammonium quaternary salt selected from those represented by the following general formula:



wherein R<sub>2</sub>, Z<sub>1</sub>, X, and e have the values set forth above.

The condensations can advantageously be carried out in the presence of a basic condensing agent, such as the trialkylamines, e. g. triethylamine, tri-n-propylamine, tri-n-butylamine etc., dialkylanilines, e. g. N,N-dimethylaniline, N,N-diethylaniline, etc., N-alkylpiperidines, e. g. N-methylpiperidine, N-ethylpiperidine, etc., heterocyclic amines, e. g. pyridine, quinoline, isoquinoline, etc., N-alkylpyrroles, e. g. N-methylpyrrole, etc.

The condensations can also be carried out in the presence of an inert solvent, such as the lower aliphatic alcohols, e. g. ethyl, n-propyl, isopropyl, n-butyl, isobutyl, etc. alcohols, diethyl ether, 1,4-dioxane, benzene, n-hexane, etc. Heat accelerates the condensations, and temperatures varying from about 25° C. to the reflux temperature of the reaction mixture can be used.

The intermediates represented by Formula III above can advantageously be prepared by heating

a compound selected from those represented by the following general formula:



wherein R, R<sub>1</sub>, n, d, L, and Z have the values given above, with an alkyl salt, such as those represented by the following general formula:



wherein R<sub>3</sub> and X<sub>1</sub> have the values set forth above. Alternatively, the intermediates represented by Formula III above can be prepared by heating a compound selected from those represented by the following general formula:



wherein R, R<sub>3</sub>, L, n, d, and Z have the values set forth above, with an alkyl salt, such as those represented by the following general formula:



wherein R<sub>1</sub> and X<sub>1</sub> have the values set forth above. The intermediates represented by Formula VI above can be prepared as described in the copending application S. N. 203,526, filed on December 29, 1950, of R. A. Jeffreys and E. B. Knott. Intermediates of the type represented by Formula VIII above have been previously described by Cook et al., "Jour. Chem. Soc." (1949), pp. 1435-7.

The following examples describe more fully the manner whereby we prepare certain of the intermediates represented by Formula III above.

Example 1.—[2-(3-ethylbenzoxazole)][4-(2-methylthio-5(4)-thiazolone)]dimethinemericyanine metho-p-toluenesulfonate



0.32 g. of [2-(3-ethylbenzoxazole)][4-(3-methyl-2-thio-2,5(3,4)-thiazoledione)]dimethinemericyanine and 0.2 g. of methyl p-toluenesulfonate were heated together for 20 minutes at 140° C. The reaction mixture set to a solid, and it was then ground to a powder and washed with dry benzene. It was recrystallized from an ethanol-diethyl ether mixture as red prisms with a blue reflex having a melting point of 222° C. It sensitized a gelatino silver chloride emulsion with a maximum at 510 m $\mu$  and a gelatino silver bromide emulsion with a maximum at 530 m $\mu$ .

Example 2.—[2-(3-ethylbenzoxazole)][4-(2-ethylthio-5(4)-thiazolone)]dimethinemericyanine metho-p-toluenesulfonate



1.0 g. of [2-(3-ethylbenzoxazole)][4-(2-ethylthio-5(4)-thiazolone)]dimethinemericyanine and 1.8 g. of methyl p-toluenesulfonate were heated together for one hour at 130° C. The resulting semi-solid was recrystallized from an

ethanol-diethyl ether mixture as flat red needles melting at 209° C.

Example 3.—[2-(3-ethylbenzoxazole)][4-(2-ethylthio-5(4)-thiazolone)]dimethinemericyanine ethiodide



2.0 g. of [2-(3-ethylbenzoxazole)][4-(2-ethylthio-5(4)-thiazolone)]dimethinemericyanine and 10 cc. of ethyl iodide were fused together in a sealed tube at 100° C. for 24 hours. The tube was then opened and the excess ethyl iodide driven off. The residue was recrystallized from ethanol as soft, rust-colored needles having a melting point of 136° C.

Example 4.—[2-(3-ethylbenzoxazole)][4-(2-ethylthio-5(4)-thiazolone)]dimethinemericyanine methomethylsulfate



1.0 g. of [2-(3-ethylbenzoxazole)][4-(2-ethylthio-5(4)-thiazolone)]dimethinemericyanine and 0.7 cc. of methyl sulfate were fused at 120° C. for 30 minutes. The crude product was then washed with diethyl ether.

Example 5.—[4-(1-ethylquinoline)][4-(2-methylthio-5(4)-thiazolone)]dimethinemericyanine metho-p-toluenesulfonate



2.0 g. of [4-(1-ethylquinoline)][4-(3-methyl-2-thio-2,5(3,4)-thiazoledione)]dimethinemericyanine and 1.2 g. of methyl p-toluenesulfonate were heated at 120° C. for 20 minutes. The solid formed was ground to a powder and then heated under reflux with benzene. The benzene was decanted off and the solid recrystallized from an ethanol-diethyl ether mixture as green flakes melting at 183° C.

Example 6.—[2-(3-ethylbenzoxazole)][4-(2-methylthio-5(4)-thiazolone)]dimethinemericyanine n-hepto-p-toluenesulfonate



1.0 g. of [2-(3-ethylbenzoxazole)][4-(3-n-heptyl-2-thio-2,5(3,4)-thiazoledione)]dimethinemericyanine and 0.5 g. of methyl p-toluenesulfonate were heated together at 120° C. for 30 minutes. The red solid obtained was ground to a powder, heated under reflux with benzene, and the benzene removed by decantation.

Example 7.—[2-(3-ethylbenzoxazole)] [4-(2-methylthio-5(4)-thiazolone)] dimethinemero-cyanine etho-p-toluenesulfonate.



4.1 g. of [2-(3-ethylbenzoxazole)] [4-(3-ethyl-2-thio-2,5(3,4)-thiaoledione)] dimethinemero-cyanine and 2.53 g. of methyl p-toluenesulfonate were heated at 120° C. for 30 minutes. The solid was ground to a powder, washed with diethyl ether, and then recrystallized from an isopropyl alcohol-diethyl ether mixture as an orange microcrystalline powder melting at 210° C. It sensitized a gelatino silver chloride emulsion with a maximum at 510 m $\mu$  and a gelatino silver bromide emulsion with a maximum at 530 m $\mu$ . 15

Example 8.—[2-(3-ethylbenzothiazole)] [4-(2-methylthio-5(4)-thiazolone)] dimethinemero-cyanine cyclohexo-p-toluenesulfonate



0.6 g. of [2-(3-ethylbenzothiazole)] [4-(3-cyclohexyl-2-thio-2,5(3,4)-thiaoledione)] dimethinemero-cyanine and 0.3 g. of methyl p-toluenesulfonate were heated together at 120° C. for 30 minutes. The solid resulting was ground to a powder and washed with diethyl ether. It was found to be deliquescent. 35

Example 9.—[2-(3-ethylbenzoxazole)] [4-(2-methylthio-5(4)-thiazolone)] dimethinemero-cyanine cyclohexo-p-toluenesulfonate



0.5 g. of [2-(3-ethylbenzoxazole)] [4-(3-cyclohexyl-2-thio-2,5(3,4)-thiaoledione)] dimethinemero-cyanine and 0.28 g. of methyl p-toluenesulfonate were heated together for 30 minutes at 120° C. The resulting solid was ground to a powder, washed with diethyl ether, and dried. It was found to be deliquescent.

Example 10.—[2-(3-ethylbenzothiazole)] [4-(2-methylthio-5(4)-thiazolone)] dimethinemero-cyanine metho-p-toluenesulfonate



4.3 g. of [2-(3-ethylbenzothiazole)] [4-(3-methyl-2-thio-2,5(3,4)-thiaoledione)] dimethinemero-cyanine and 2.9 g. of methyl p-toluenesulfonate were heated together at 130° C. for 30 minutes. The solid product was ground to a powder, washed with diethyl ether. On recrystallization from an ethanol-diethyl ether mixture, it was obtained as maroon leaflets melting at 182° C. (6.2 g.). It sensitized both a gelatino silver chlorobromide emulsion and a gelatino silver bromide emulsion with a maximum at 570 m $\mu$ . 65

Example 11.—[2-(3-ethylbenzothiazole)] [4-(2-ethylthio-5(4)-thiazolone)] dimethinemero-cyanine methomethylsulfate



3.48 g. of [2-(3-ethylbenzothiazole)] [4-(2-ethylthio-5(4)-thiazolone)] dimethinemero-cyanine (Cook et al., "Jour. Chem. Soc." (1949), pp. 1435-6) and 1.9 g. of methyl sulfate were heated together at 120° C. for 15 minutes. The resulting solid was ground to a powder and then washed with diethyl ether.

Example 12.—[2-(3-methylthiazoline)] [4-(2-ethylthio-5(4)-thiazolone)] dimethinemero-cyanine methomethylsulfate



30 The following examples illustrate the manner whereby certain of the intermediates represented by Formula VIII above can be prepared.

Example 13.—[2-(3-ethylbenzoxazole)] [4-(2-ethylthio-5(4)-thiazolone)] dimethinemero-cyanine



45 9.0 g. of N-(dithiocarbethoxy)glycine, 40 cc. of acetic anhydride, and 12 cc. of ethyl orthoformate were heated together on a steam bath for 30 minutes. The unreacted liquids were then distilled off and the residual oil consisting of 2-ethylthio-4-ethoxymethylene-5(4)-thiazolone was refluxed for five minutes with 14.5 g. of 2-methylbenzoxazole ethiodide, 40 cc. of ethanol, and 10 cc. of triethylamine, and the reaction mixture then chilled. The resulting dye after recrystallization from ethanol formed flat, steel-blue needles melting at 156° C.

50 Example 14.—[2-(3-methylthiazoline)] [4-(2-ethylthio-5(4)-thiazolone)] dimethinemero-cyanine



55 This dye was prepared in the same manner as the dye of Example 13 by replacing the 2-methylbenzoxazole ethiodide by a molecularly equivalent amount of 2-methylthiazoline methiodide. The desired product was obtained as maroon needles melting at 129° C. from ethanol.

60 The following examples will serve to illustrate the manner whereby we prepare our new tri-nuclear dyes.

Example 15.—[2-(3-ethylbenzoxazole)] [4-(5-oxo-2-phenyl-4-oxazolinylidene)-3-methyl-5-(4-thiazolidone)] dimethinecyanine



0.5 g. of the quaternary salt obtained in Example 1 above and 0.18 g. of 2-phenyl-5(4)-oxazolone were heated under reflux for four hours in the presence of 10 cc. of ethanol and 0.15 cc. of triethylamine. The reaction mixture was chilled and the solid filtered off. The dye was recrystallized from a pyridine-diethyl ether mixture as small bluish needles melting at 310° C. It sensitized a gelatino silver chloride emulsion with maxima at 540 and 570 m $\mu$  and a gelatino silver bromide emulsion with a maximum at 610 m $\mu$ .

Example 16.—{2-(3-ethylbenzoxazole)} {2-[4-(2-[3-ethylbenzoxazolinylidene] ethylidene)-3-methyl-5(4)-thiazolone]} methinecyanine iodide



0.5 g. of the quaternary salt obtained in Example 1 above, 0.3 g. of 2-methylbenzoxazole ethiodide, 0.15 cc. of triethylamine, and 10 cc. of ethanol were heated under reflux for 4 hours. The reaction mixture was chilled and the precipitate filtered off. The dye, as recrystallized from methanol, melted at 300° C. and was obtained as grey prisms. It sensitized a gelatino silver chloride emulsion with maxima at 540 and 590 m $\mu$  and a gelatino silver bromide emulsion with a maximum at 590 m $\mu$ .

Example 17.—{2-(3-ethylbenzothiazole)} {2-[4-(2-[3-ethylbenzoxazolinylidene] ethylidene)-3-methyl-5(4)-thiazolone]} methinecyanine iodide



0.3 g. of the quaternary salt obtained in Example 1 above, 0.2 g. of 2-methylbenzothiazole ethiodide, 0.12 cc. of triethylamine, and 6 cc. of ethanol were refluxed together for one hour, chilled, and the reaction mixture filtered. The dye was recrystallized from pyridine as green needles melting at 286° C. It sensitized a gelatino silver chloride emulsion with maxima at 520 and 600 m $\mu$  and a gelatino silver bromide emulsion with a maximum at 630 m $\mu$ .

Example 18.—{2-(3-methylthiazoline)} {2-[4-(2-[3-ethylbenzoxazolinylidene] ethylidene)-3-methyl-5(4)-thiazolone]} methinecyanine iodide



0.3 g. of the quaternary salt obtained in Ex-

ample 1 above, 0.15 g. of 2-methylthiazoline methiodide, 0.12 cc. of triethylamine, and 6 cc. of ethanol were refluxed for one hour, chilled, and then filtered. The desired dye was recrystallized from methanol as red-bronze prisms melting at 298° C. It sensitized a gelatino silver chloride emulsion with maxima at 520 and 570 m $\mu$  and a gelatino silver bromide emulsion with a maximum at 590 m $\mu$ .

Example 19.—[4-(1-ethylquinoline)] {2-[4-(1-ethyl-1,4-dihydroquinolinylidene)ethylidene]3-methyl-5(4)-thiazolone} methinecyanine iodide



0.51 g. of the quaternary salt obtained in Example 5 above, 0.3 g. of lepidine ethiodide, 0.2 cc. of triethylamine, and 10 cc. of ethanol were refluxed together for one hour on the steam bath. The reaction mixture was then chilled, and the precipitate collected on a filter. After recrystallization from aniline, the dye was obtained as a dark olive-green powder having a melting point of 234° C.

Example 20.—[2-(1-ethylquinoline)] {2-[4-(2-[3-ethylbenzoxazolinylidene]ethylidene)-3-n-heptyl-5(4)-thiazolone]} methinecyanine iodide



0.5 g. of the quaternary salt obtained in Example 6 above, 0.26 g. of quinaldine ethiodide, 0.2 cc. of triethylamine, and 5 cc. of ethanol were refluxed together on a steam bath for one hour, and the reaction mixture then chilled. The precipitate was collected on a filter and then recrystallized from a methanol-diethyl ether mixture. It was obtained as lustrous green prisms melting at 244° C. It sensitized a gelatino silver bromide emulsion from 570 to 710 m $\mu$ .

Example 21.—[4-(1-ethylquinoline)] {2-[4-(2-[3-ethylbenzoxazolinylidene]ethylidene)-3-n-heptyl-5(4)-thiazolone]} methinecyanine iodide



0.5 g. of the quaternary salt obtained in Example 6 above, 0.26 g. of lepidine ethiodide, 0.2 cc. of triethylamine, and 5 cc. of ethanol were heated on a steam bath for 6 hours and the reaction mixture then chilled. The precipitate was filtered off, and then recrystallized from a methanol-diethyl ether mixture as small moss-green needles melting at 184° C. It sensitized a gel-

## 11

tino silver bromiodide emulsion with maxima at 640 and 700 m $\mu$ .

Example 22.—[2-(3-ethylbenzothiazole)] {4-[2-(3-ethyl-4-oxo-2-thio-5-thiazolidinylidene)-3-cyclohexyl-5(4)-thiazolidone]} dimethinemeroxyanine



0.9 g. of the quaternary salt obtained in Example 8 above, 0.25 g. of 3-ethylrhodanine, 0.2 cc. of triethylamine and 10 cc. of ethanol were refluxed on a steam bath for one hour, and the mixture chilled. The precipitate was collected on a filter and recrystallized from a benzene-petroleum ether mixture as grass-green needles melting at 239° C. It sensitized a gelatino silver chloride emulsion with maxima at 470 and 650 m $\mu$ , and a gelatino silver bromiodide emulsion with a flat maximum lying between 620 and 680 m $\mu$ .

Example 23.—[2-(3-ethylbenzoxazazole)] {4-[2-(5-oxo-2-n-octythio-4-thiazolinylidene)-3-cyclohexyl-5-thiazolidone]} dimethinemeroxyanine



0.45 g. of N-(dithiocarbo-n-octyloxy)glycine were dissolved in 5 cc. of acetic anhydride and then heated for 30 minutes on a steam bath. The unreacted acetic anhydride and acetic acid formed during the reaction were removed under a vacuum. To the residual oil (2-ethylthio-5(4)-thiazolone) were added 0.86 g. of the quaternary salt obtained in Example 9 above, 0.3 cc. of triethylamine, and 10 cc. of ethanol, and the resulting solution was heated on a steam bath for 30 minutes and then chilled. The precipitate was collected on a filter and recrystallized from ligroin as yellow-green prisms melting at 150° C. It sensitized a gelatino silver chloride emulsion with maxima at 400 and 590 m $\mu$  and a gelatino silver bromiodide emulsion with a maximum at 610 m $\mu$ .

Example 24.—[2-(3-methylbenzothiazole)] {2-[4-(2-(3-ethylbenzoxazolinylidene)ethylidene)-3-ethyl-5-thiazolidone]} azamethinecyanine p-toluenesulfonate



1.0 g. of the quaternary salt obtained in Example 7 above, 0.32 g. of 2-imino-3-methylbenzothiazoline, 0.15 cc. of triethylamine, and 6 cc. of ethanol were heated for 2 hours on a steam bath. The reaction mixture was chilled, and the precipitate collected on a filter. The dye product recrystallized from isopropanol as a red microcrystalline powder melting at 196° C. It sensitized a gelatino silver chloride emulsion with maxima at 400 and 560 m $\mu$ , and a gelatino silver bromiodide emulsion with a maximum at 580 m $\mu$ .

## 12

Example 25.—{2-(3-ethylbenzothiazole)} {4-[2-(3-methyl-5-oxo-2-thio-4-thiazolidinylidene)-3-methyl-5-thiazolidone]} dimethinemeroxyanine



1.04 g. of the quaternary salt obtained in Example 10 above, 0.29 g. of 3-methyl-2-thio-5-thiazolidone (Cook et al., "Jour. Chem. Soc." (1949), page 2340), 0.2 cc. of triethylamine, and 10 cc. of ethanol were heated on a steam bath for 20 minutes, and then chilled. The precipitate was collected on a filter (0.8 g.) and recrystallized from a chloroform-petroleum ether mixture as a dark-green microcrystalline powder melting at 274° C. It sensitized both gelatino-silver chlorobromide and silver bromide emulsions with a maximum at 580 m $\mu$ .

Example 26.—{2-(3-ethylbenzothiazole)} {4-[2-(3-ethyl-4-oxo-2-thio-5-thiazolidinylidene)-3-methyl-5-thiazolidone]} dimethinemeroxyanine



1.04 g. of the quaternary salt obtained in Example 10 above, 0.32 g. of 3-ethylrhodanine, 0.2 cc. of triethylamine, and 10 cc. of ethanol were heated on a steam bath for 20 minutes and then chilled. The precipitate was collected on a filter (1.0 g.) and recrystallized from pyridine as long indigo needles, melting at 300° C. It sensitized a gelatino silver chlorobromide emulsion with a maximum at 670 m $\mu$ .

Example 27.—{2-(3-ethylbenzothiazole)} {4-[2-(5-oxo-2-n-octythio-4-thiazolinylidene)-3-methyl-5-thiazolidone]} dimethinemeroxyanine



0.54 g. of N-(thiocarbo-n-octyloxy)glycine and 5 cc. of acetic anhydride were heated together on a steam bath for 30 minutes. The unreacted acetic anhydride and acetic acid formed during the reaction were removed under a vacuum. To the residual oil consisting of 2-n-octythio-5(4)-thiazolone were added 1.04 g. of the quaternary salt obtained in Example 10 above 0.3 cc. of triethylamine and 10 cc. of ethanol, and the mixture heated on a steam bath for 20 minutes and then chilled. The dye which separated weighed 0.9 g. and was recrystallized from a benzene-petroleum ether mixture as lustrous green leaflets melting at 155° C. It sensitized a gelatino silver chlorobromide emulsion with maxima at 580 and 640 m $\mu$ .

Example 28.—{4-(1-ethylquinoline)}{2-[4-(2-[3-ethylbenzoxazolinylidene]ethylidene)-3-ethyl-5-thiazolidone]}methinecyanine iodide



0.488 g. of the quaternary salt obtained in Example 3 above, 0.299 g. of lepidine ethiodide, 0.2 cc. of triethylamine, and 10 cc. of ethanol were refluxed for 30 minutes, and the solution then chilled. The precipitate (0.4 g.) was collected on a filter and recrystallized from a methanol-diethyl ether mixture as glittering blue-black crystals melting at 272° C. It sensitized a gelatino silver chloride emulsion with a maximum at 670 m $\mu$ .

Example 29.—{2-(3-ethylbenzothiazole)}{2-[4-(2-[3-ethylbenzoxazolinylidene]ethylidene)-3-methyl-5-thiazolidone]}methinecyanine iodide.



1.6 g. of the quaternary salt obtained in Example 2 above, 0.9 g. of 2-methylbenzothiazole ethiodide, 0.5 cc. of triethylamine, and 10 cc. of ethanol were refluxed for 30 minutes and then chilled. The precipitate (0.9 g.) was collected on a filter and recrystallized from pyridine as fine green needles melting at 292° C. It sensitized a gelatino silver chloride emulsion with a maximum at 600 m $\mu$  and a gelatino silver bromide emulsion with a maximum at 630 m $\mu$ .

Example 30.—{2-(3-ethylbenzoxazole)}{2-[4-(2-[3-ethyl-4-oxo-2-thio-5-thiazolidinylidene]-3-methyl-5-thiazolidone]}dimethine-merocyanine.



1.03 g. of the quaternary salt obtained in Example 2 above, 0.3 g. of 3-ethylrhodanine, 0.3 cc. of triethylamine and 10 cc. of ethanol were refluxed for 10 minutes, and then cooled. The precipitate was collected on a filter and recrystallized from pyridine as fine mauve needles melting above 310° C. It sensitized a gelatino silver chloride emulsion with a maximum at 600 m $\mu$  and a gelatino silver bromide emulsion with a maximum at 630 m $\mu$ .

Example 31.—{2-(3-ethylbenzothiazole)}{2-[4-(2-[3-ethyl-4-oxo-2-thio-5-thiazolidinylidene]-3-ethyl-5-thiazolidone]}dimethine-merocyanine.



1.74 g. of [2-(3-ethylbenzothiazole)]{4-(2-ethylthio-5(4)-thiazolone)} dimethinemerocya-

nine and 0.77 g. of ethyl sulfate were fused at 120 to 130° C. for 4 hours, and the resulting solid boiled out with benzene. There were then added 0.75 g. of 3-ethylrhodanine, 1.0 cc. of triethylamine, and 10 cc. of ethanol, and the solution refluxed for 20 minutes, and then chilled. The precipitate was collected on a filter and recrystallized from pyridine as gold-green crystals melting at 292° C. It sensitized a gelatino silver chloride emulsion with a maximum at 650 m $\mu$  and a gelatino silver bromide emulsion with a maximum at 670 m $\mu$ .

Example 32.—{2-(3-ethylbenzoxazole)}{4-[2-(3-ethyl-4-oxo-2-thio-5-thiazolidinylidene)-3-ethyl-5-thiazolidone]}dimethinemerocyanine



1.0 g. of [2-(3-ethylbenzoxazole)]{4-(2-ethylthio-5(4)-thiazolone)} dimethinemerocyanine and 0.5 g. of ethyl sulfate were fused at 130° C. for 4 hours, and 0.45 g. of 3-ethylrhodanine, 0.5 cc. of triethylamine and 10 cc. of ethanol were added. The solution was refluxed for 10 minutes, and then chilled. The precipitate was collected on a filter and recrystallized from benzene as steel-blue needles melting at 278° C. It sensitized a gelatino silver chloride emulsion with a maximum at 600 m $\mu$  and a gelatino silver bromide emulsion with a maximum at 625 m $\mu$ .

Example 33.—{2-(3-ethylbenzoxazole)}{2-[4-(2-[3-ethylbenzothiazolinylidene]ethylidene)-3-methyl-5-thiazolidone]} methinecyanine iodide



1.2 g. of the quaternary salt obtained in Example 11 above, 0.7 g. of 2-methylbenzoxazole ethiodide, 0.5 cc. of triethylamine, and 10 cc. of ethanol were refluxed for 10 minutes, and then chilled. The precipitate was collected on a filter and on recrystallization was obtained as golden-green needles melting at 280° C. It sensitized a gelatino silver chloride emulsion with a maximum at 610 m $\mu$  and a gelatino silver bromide emulsion with a maximum at 635 m $\mu$ .

Example 34.—{4-(1-ethylquinoline)}{2-[4-(2-[3-ethylbenzothiazolinylidene]ethylidene)-3-methyl-5-thiazolidone]} methinecyanine iodide



1.2 g. of the quaternary salt obtained in Example 11 above, 0.8 g. of lepidine ethiodide, 0.5 cc. of triethylamine, and 10 cc. of ethanol were refluxed for 10 minutes and then cooled. The precipitate was collected on a filter and washed with ethanol until the washings were blue. The precipitate was then boiled out several times with

fresh portions of methanol. It formed green needles melting at 292° C.

*Example 35.*—{2-(3-ethylbenzothiazole)} {2-[4-(2-3-ethylbenzothiazolinylidene) ethylidene]-3-methyl-5-thiazolidone} methinecyanine iodide



1.2 g. of the quaternary salt obtained in Example 11 above, 0.8 g. of 2-methylbenzothiazole ethiodide, 0.5 cc. of triethylamine, and 10 cc. of ethanol were refluxed for 10 minutes and then cooled. The precipitate was collected on a filter, and washed with ethanol until the washings were blue. It was then boiled out several times with fresh portions of methanol. It formed green needles melting at 278° C. It sensitized a gelatino silver bromide emulsion with a maximum at 660 m $\mu$ .

*Example 36.*—{2-(3-ethylbenzothiazole)} {4-[2-(2-n-heptylthio - 5-oxo-4-thiazolinylidene)-3-methyl - 5 - thiazolidone]dimethinememerocyanine



0.7 g. of N-(dithiocarbo-n-heptoxy) glycine and 7 cc. of acetic anhydride were heated for 30 minutes on a steam bath, and the unreacted acetic anhydride and acetic acid formed during the reaction removed under a vacuum. To the residue consisting of 2-n-heptylthio-5(4)-thiazolone were added 1.2 g. of the quaternary salt obtained in Example 11 above, 0.5 cc. of triethylamine, and 10 cc. of ethanol, and the solution was refluxed for 5 minutes and chilled. The precipitate was collected on a filter and recrystallized from benzene as fine green needles melting at 200° C. It sensitized a gelatino silver bromide emulsion with a maximum at 645° C.

The N-(dithiocarbo-n-octoxy) glycine used in Example 23 above was prepared as follows:

*Example 37.*—N-(dithiocarbo-n-octoxy) glycine



22.4 g. of potassium hydroxide were dissolved in 50 cc. of water and the solution chilled. There were then added 15.0 g. of glycine and 15.2 g. of carbondisulfide, and the whole shaken mechanically until a clear orange solution resulted. A solution of 38.6 g. of n-octylamine in 50 cc. of ethanol was added, and the mixture heated for 30 minutes on a steam bath. To the resulting one-phase solution there were added 100 cc. of water, and the cloudiness resulting removed by extraction with diethyl ether. The aqueous layer was warmed gently under reduced pressure to expel any dissolved ether, the solution chilled, and acidified with concentrated hydrochloric acid. The precipitate was collected on a filter, washed with water, air-dried, and recrystallized from petroleum ether (B. P. 60-80° C.) as glistening plates melting at 100° C.

By replacing the n-octylamine in Example 37 can be obtained.

by a molecularly equivalent amount of n-heptylamine, N-(dithiocarbo-n-heptoxy) glycine was obtained as glistening, waxy plates melting at 99° C. on recrystallization from petroleum ether.

The N-(thiocarbo-n-octoxy) glycine used in Example 27 above was prepared as follows:

*Example 38.*—N-thiocarbo-n-octoxy) glycine



1 g. mol. of n-octyl alcohol was dissolved in 250 cc. of carbondisulfide and 1 g. mol. of powdered potassium hydroxide was added. The whole was shaken mechanically until it had set to a solid. After chilling overnight, the salt was collected, washed with diethyl ether, and air-dried.

1 g. mol. of the potassium n-octoxydithioformate (potassium n-octylzanthate) was added to 250 cc. of methanol, and 1 g. mol. of ethylbromide added. The mixture was warmed for several minutes, and water added. The oil which separated was taken up in diethyl ether, dried over sodium sulfate, and the ether removed by warming under a vacuum.

1 g. mol. of the ethyl n-octoxydithioformate (ethyl n-octylzanthate) thus obtained, 1 g. mol. of glycine, 1 g. mol. of potassium hydroxide were added to 200 cc. of a 50 per cent aqueous ethanol solution, and the whole refluxed on a steam bath for 18 hours. The solution was then concentrated to 100 cc., 100 cc. of water was added, and the solution made acid with hydrochloric acid. The precipitate of the desired 2-n-octoxy-5(4)-thiazolone was recrystallized from petroleum ether as fine needles melting at 72° C.

Operating in a similar manner to that illustrated in the above examples, other trinuclear dyes can be prepared according to our invention. For example, by replacing the quaternary salt used in Example 15 by a molecularly equivalent amount of [2-(3-methylbenzothiazole)] [4-(2-methylthio - 5(4) - thiazolone)] merocyanine metho-p-toluenesulfonate, [2-(3-methylbenzothiazole)] [4-(5-oxo-2-phenyl - 4-oxazolinylidene)-3-methyl-5(4)-thiazolidone] merocyanine represented by the following formula:



can be obtained.

In like manner, by replacing the quaternary salt used in Example 18 above, by a molecularly equivalent amount of [2-(3-ethylbenzoxazole)] [4-(2-methylthio - 5(4) - thiazolone)] tetramethinememerocyanine metho-p-toluenesulfonate, [2-(3-methylthiazoline)] {2-[4-(2-ethylbenzoxazolylidene) - 1,3-butadienylidene]-3-methyl-5(4)-thiazolone} methinecyanine iodide represented by the following formula:



As shown above we have found that our new dyes spectrally sensitive photographic silver halide emulsions when incorporated therein. The dyes are especially useful for extending the spectral sensitivity of the customarily employed gelatino-silver-chloride, gelatino-silver-chlorobromide, gelatino-silver-bromide and gelatino-silver bromiodide developing-out emulsions. To

consisting of those represented by the following general formulas:



and



20 prepare emulsions sensitized with one or more of our new dyes, it is only necessary to disperse the dye or dyes in the emulsions. The methods of incorporating dyes in emulsions are simple and are known to those skilled in the art. In practice, it is convenient to add the dyes to the emulsions in the form of a solution in an appropriate solvent. Methanol or acetone has proved satisfactory as a solvent for most of our new dyes. Where the dyes are quite insoluble in methyl alcohol, a mixture of acetone and pyridine is advantageously employed as a solvent. The dyes are advantageously incorporated in the finished, washed emulsions and should be uniformly distributed throughout the emulsions. The particular solvent used will, of course, depend on the solubility properties of the particular dye.

25 The concentration of the dyes in the emulsions can vary widely, e. g. from 5 to 100 mg. per liter of flowable emulsion. The concentration of the dyes will vary according to the type of emulsion and according to the effect desired. The suitable and most economical concentration for any given emulsion will be apparent to those skilled in the art, upon making the ordinary tests and observations customarily used in the art of emulsion making. To prepare a gelatino-silver-halide emulsion sensitized with one or more of our new dyes, the following procedure is satisfactory:

30 A quantity of dye is dissolved in methyl alcohol or acetone (or a mixture of acetone and pyridine) and a volume of this solution, which may be diluted with water, containing from 5 to 100 mg. of dye, is slowly added to about 1000 cc. of gelatino-silver-halide emulsion, with stirring. Stirring is continued until the dye is thoroughly dispersed in the emulsion.

35 With most of our dyes, from 10 to 20 mg. of dye per liter of gelatino-silver-bromide or bromiodide emulsion (containing about 40 g. of silver halide) suffices to produce the maximum sensitizing effect. With the finer grain emulsions, somewhat larger concentration of dye may be needed to produce the maximum sensitizing effect.

40 The above statements are only illustrative, as it will be apparent that the dyes can be incorporated in photographic emulsions by any of the other methods customarily employed in the art, e. g. by bathing a plate or film upon which an emulsion is coated in a solution of the dye in an appropriate solvent. However, bathing methods are ordinarily not to be preferred. Emulsions sensitized with the dyes can be coated on suitable supports, such as glass, cellulose derivative film, resin film or paper in the usual manner.

45 What we claim as our invention and desire secured by Letters Patent of the United States is:

1. A trinuclear dye selected from the group

75

wherein  $R$ ,  $R_1$ , and  $R_2$  each represents an alkyl group of the formula  $C_mH_{2m+1}$  wherein  $m$  represents a positive integer of from 1 to 8,  $L$  represents a methine group,  $a$  and  $n$  each represents a positive integer from 1 to 2,  $d$  represents a positive integer from 1 to 3,  $X$  represents an anion,  $Q$  represents the non-metallic atoms necessary to complete a heterocyclic nucleus containing 5 atoms in the heterocyclic ring, 3 of said atoms being carbon atoms, 1 of said atoms being a nitrogen atom, and the other of said atoms being selected from the group consisting of an oxygen atom, a sulfur atom, and a nitrogen atom, and  $Z$  and  $Z_1$  each represents the non-metallic atoms necessary to complete a heterocyclic nucleus selected from the group consisting of those of the thiazole series, those of the benzothiazole series, those of the naphthothiazole series, those of the oxazole series, those of the benzoxazole series, 35 those of the naphthoxazole series, those of the selenazole series, those of the benzoselenazole series, those of the naphthoselenazole series, those of the thiazoline series, those of the 2-quinoline series, those of the 4-quinoline series, 40 those of the 1-isoquinoline series, those of the 3-isoquinoline series, those of the pyridine series, and those of the 3,3-dimethylindolenine series.

2. The trinuclear dye represented by the following formula:



50 3. The trinuclear dye represented by the following formula:



55 4. The trinuclear dye represented by the following formula:



60 5. The trinuclear dye represented by the following formula:



19

6. The trinuclear dye represented by the following formula:



7. A process for preparing a trinuclear dye comprising condensing a cyclammonium quaternary salt selected from those represented by the following general formula:



wherein R, R<sub>1</sub>, and R<sub>2</sub> each represents an alkyl group of the formula C<sub>n</sub>H<sub>2m+1</sub>, wherein m represents a positive integer from 1 to 8; X<sub>1</sub> represents an anion, n represents a positive integer from 1 to 2, d represents a positive integer from 1 to 3; and Z represents the non-metallic atoms necessary to complete a heterocyclic nucleus selected from the group consisting of those of the thiazole series, those of the benzothiazole series, those of the oxazole series, those of the benzoxazole series, those of the naphthoxazole series, those of the selenazole series, those of the benzoselenazole series, those of the thiazoline series, those of the 2-quinoline series, those of the 4-quinoline series, those of the 1-isoquinoline series, those of the 3-isoquinoline series, those of the pyridine series, and those of the 3,3-dimethylindolenine series.

20 25 30 35 40

atoms being carbon atoms, 1 of said atoms being a nitrogen atom, and the other of said atoms being selected from the group consisting of an oxygen atom, a sulfur atom and a nitrogen atom; and cyclammonium quaternary salt selected from those represented by the following general formula:



wherein R<sub>2</sub> represents an alkyl group of the formula C<sub>n</sub>H<sub>2m+1</sub> wherein m represents a positive integer from 1 to 8, X represents an anion, e represents a positive integer from 1 to 2, and Z<sub>1</sub> represents the non-metallic atoms necessary to complete a heterocyclic nucleus selected from the group consisting of those of the thiazole series, those of the benzothiazole series, those of the naphthothiazole series, those of the oxazole series, those of the benzoxazole series, those of the naphthoxazole series, those of the selenazole series, those of the benzoselenazole series, those of the naphthoselenazole series, those of the thiazoline series, those of the 2-quinoline series, those of the 4-quinoline series, those of the 1-isoquinoline series, those of the 3-isoquinoline series, those of the pyridine series, and those of the 3,3-dimethylindolenine series.

8. A process according to claim 7, wherein the condensation is performed in the presence of triethylamine.

PER AUBERT,  
ROY A. JEFFREYS,  
EDWARD B. KNOTT.

References Cited in the file of this patent

UNITED STATES PATENTS

| Number:   | Name:   | Date:         |
|-----------|---------|---------------|
| 2,170,804 | Brooker | Aug. 29, 1939 |
| 2,388,962 | Ery     | Nov. 13, 1945 |

OTHER REFERENCES

Cook, J. Chem. Soc. (1948), pp. 1056-1057.  
Cook, J. Chem. Soc. (1949), pp. 1425-1437,  
2342-2346.



wherein Q represents the non-metallic atoms necessary to complete a heterocyclic nucleus containing 5 atoms in the heterocyclic ring, 3 of said